

# United States Patent [19]

Muta et al.

[11] 3,912,959

[45] Oct. 14, 1975

[54] **HIGH PRESSURE SODIUM VAPOR  
DISCHARGE LAMPS**

[75] Inventors: **Akinori Muta; Yasuo Tsukuda**, both of Tokyo, Japan

[73] Assignee: **Hitachi, Ltd.**, Japan

[22] Filed: **Mar. 16, 1973**

[21] Appl. No.: **341,849**

[30] **Foreign Application Priority Data**

Mar. 16, 1972 Japan..... 47-26807

[52] U.S. Cl..... **313/220; 313/221**

[51] Int. Cl. .... **H01j 61/30**

[58] **Field of Search**..... 313/221, 220

[56] **References Cited**

UNITED STATES PATENTS

3,363,134 1/1968 Johnson..... 313/221

*Primary Examiner*—Rudolph V. Rolinec  
*Assistant Examiner*—Darwin R. Hostetter  
*Attorney, Agent, or Firm*—Craig & Antonelli

[57]

## ABSTRACT

A ceramic tube consisting of sintered high transparent polycrystalline yttria is used as an envelope in a high pressure sodium vapor discharge lamp.

The discharge lamp having this envelope excels in operation for a long period of time because the transparency of this envelope is not reduced at all when it is exposed to saturated sodium vapor at elevated temperatures.

**7 Claims, 4 Drawing Figures**



FIG. I



FIG. 2



FIG. 3



FIG. 4



## HIGH PRESSURE SODIUM VAPOR DISCHARGE LAMPS

### BACKGROUND OF THE INVENTION

This invention relates to high pressure sodium vapor discharge lamps generally and more particularly to such lamps which use a ceramic envelope consisting of a sintered highly transparent polycrystalline yttrium oxide.

Conventionally, a transparent polycrystalline alumina pipe was used as an envelope in a high pressure metal vapor discharge lamp. This material has a total transmission of approximately 90 percent; and, when used as an envelope in a high pressure sodium vapor discharge lamp, it has a radiation efficiency of approximately 100  $lm/W$ , which is lower than that of a low pressure sodium vapor discharge lamp. In addition, among the materials enclosed within the envelope, sodium is decreased gradually in its quantity, if the lamp is illuminated for a long time. Since the alumina of the envelope begins to evaporate and is changed into an oxide of lower valence as the temperature on the wall of the envelope exceeds 1400°C, the outer envelope is observed to blacken on its inner wall. The transparent polycrystalline body produced by sintering a mixture of yttria ( $Y_2O_3$ ) and thoria ( $ThO_2$ ) produced and marketed by General Electric Company, U.S.A., under the trade name of Yttralox shows excellent transmissivity, but it is blackened when the body is heated in a sodium vapor atmosphere.

### SUMMARY OF THE INVENTION

An object of this invention is to obviate these drawbacks in high pressure sodium vapor discharge lamps and to provide a high pressure sodium vapor discharge lamp having a higher radiation efficiency and a lesser reduction in the quantity of sodium enclosed within the envelope, in addition to a reduction in blackening of the inner wall of the outer envelope and a longer service life.

According to the present invention, the above object is attained by the use of a transparent polycrystalline yttria ceramic tube as an envelope in a high pressure sodium vapor discharge lamp. By this means, the radiation efficiency can be increased to 116 to 124  $lm/W$ , with suppression of the decrease in sodium quantity within the envelope and the blackening of the inner wall of the outer envelope at higher than 1400°C, while the service life of the discharge lamp can be prolonged.

### BRIEF DESCRIPTION OF THE DRAWING

FIG. 1 is a plan view of the high pressure sodium vapor discharge lamp according to this invention using a transparent polycrystalline yttria ceramic tube as an envelope; and

FIG. 2 is a diagram showing the relation between the grain size and the in-line transmission of the yttria sintered body; and

FIGS. 3 and 4 are detailed cross-sectional views of alternative embodiments of the high pressure sodium vapor discharge lamp in accordance with the present invention.

### DESCRIPTION OF THE PREFERRED EMBODIMENTS

Preferred embodiments of the present invention will now be described below.

FIG. 1 shows, in plan view, a high pressure sodium vapor discharge lamp according to the present invention, including a tubular elongated envelope 1 made of transparent yttria and sealed at both ends by niobium caps 4 and 5 with the use of a glass material consisting of, for example, 55 percent alumina, 39 percent calcia and 6 percent magnesia, said niobium caps carrying internal electrodes 2 and 3. The envelope 1 is filled with an amalgam of 30 percent sodium sodium vapor and

10 Xenon at a pressure of 20 mm Hg. The envelope 1 is suspended in the conventional manner in an outer envelope 10 made of hard glass in which is provided electrical leads 6 and 7, connected in the known manner to a socket 8, as well as the standard getter rings 9. High 15 vacuum pressure is maintained inside the outer envelope 10.

Basically, the transparent yttria envelope 1 according to this invention is produced by the process comprising the steps of

20 1. Providing finely powdered yttrium oxide of high purity;

2. Pressure molding said powders into a tubular body and, if desired, subjecting the latter to a vacuum degassing operation; and

25 3. Heating the molded body for more than 10 minutes at a temperature of 1950° to 2400°C under an atmosphere of hydrogen or oxygen, or in a vacuum.

The purity of the powdered material can be varied, depending upon the usage of the powdered material or

30 the property of the impurities mixed into the material. For instance, in cases where the sintered body is used as an envelope, a window, or a lens in an optical system required to be heat resistant and have a high transparency, it is necessary to maintain the purity approximately higher than 99.99 percent and, above all, to avoid the mixture of terbium, molybdenum and other coloring impurities into the sintered body as much as possible.

The powdered material with grain sizes less than 30 $\mu$  40 may safely be employed, but a powdered material having grain sizes as small as possible, especially grain sizes in the range of 0.2 to 1.0 $\mu$ , is preferred from the practical point of view.

A hydraulic press, for instance, can be used for pressure molding the powdered material. While the molding pressure is not so critical, sinterability tends to abruptly decrease with molding pressures less than 0.2 ton/cm<sup>2</sup>. Therefore, a molding pressure higher than 0.2 ton/cm<sup>2</sup> is preferred. Sinterability can be increased by 45 using a higher molding pressure, however, when the pressure is increased excessively, the density of the sintered body may be occasionally lowered, due to the expansion of the pores of the sintered body occurring at the time of sintering. Therefore, when the molding operation is carried out under a higher molding pressure, it is necessary to use a lower press speed or an atmosphere of reduced pressure, or it is necessary to subject the molded body to degassing by heating the latter in 50 an atmosphere of reduced pressure so that the gas included in the molded body can be reduced as much as possible. Expansion of the sintered body can also be prevented to a limited extent by using a reduced heating speed in the sintering process.

With a molding pressure higher than 8 to 9 tons/cm<sup>2</sup>, 55 it is necessary to carry out a degassing operation as described above, except where an extremely low press speed is employed. With a molding pressure higher

than 25 to 30 tons/cm<sup>2</sup>, increased molding pressures can hardly be expected to bring about an increase in sinterability and, in addition, the above-mentioned degassing operation can be effected only with considerable difficulty. Therefore, it is usually preferred to use a molding pressure less than 30 ton/cm<sup>2</sup>. For instance, when the pressure of 7 to 10 tons/cm<sup>2</sup> is used for a molding operation continuing for 10 minutes, a degassing operation is preferably carried out for about one hour under a vacuum pressure of 10<sup>-2</sup> mm Hg while heating to 100° to 200° C. When the molding pressure of 20 to 30 tons/cm<sup>2</sup> is used, a degassing operation is preferably carried out for more than 1 hour under a vacuum pressure of 10<sup>-3</sup> mm Hg while heating to higher than 210° C.

The heating atmosphere used in the sintering process is not strictly limited and may be selected depending on the type of heater used in the heating furnace. Thus, with the use of an oxide or high-melting metal heater, an oxygen atmosphere of a hydrogen or vacuum atmosphere may be used, respectively.

Especially, if desired to readily and completely remove the pores from crystal grains of yttrium oxides, dry hydrogen having a dew point approximately below -20° C may be preferably employed as an atmosphere to introduce oxygen defects into the yttrium oxide grains. It is to be noted that, when the heating is carried out under such an atmosphere for a long time, the sintered body is colored black partially or in its entirety. In this case, a colorless product can be obtained if the sintered body is re-heated in a humid or wet hydrogen atmosphere having a dew point in the range of 0° C to room temperature.

While the sintering temperature and time vary slightly depending on the sintering atmosphere, for example, it is necessary to heat the mixture for more than 10 minutes at a temperature higher than 1950° C. While the upper limit of the sintering temperature is 2400° C, which is slightly below the melting point of yttria, the mixture is preferably heated for more than 45 minutes at a temperature of 2000° to 2300° C, if desired to obtain a sintered body having high density and good transparency as well as uniform structure utilizable with the present invention.

Table 1 shows the result of sodium resistance tests on the transparent yttria prepared by the above process, as well as transparent alumina prepared by the conventional process and commercially available Yttrolox. These sodium resistance tests were carried out in a way such that each sample was enclosed in a sodium-sealed niobium tube in which saturated sodium vapor is introduced and the tube was then heated under the conditions shown in the Table.

A similar high pressure sodium vapor discharge lamp, such as described in conjunction with FIG. 1, was produced with the use of a transparent alumina tube as the envelope 1, and a comparative test was carried out under lighted conditions with this discharge lamp and the product of the present invention.

It was observed that, with the use of the conventional alumina tube as the envelope, the inner wall of the outer envelope 10 began to blacken as the temperature of the envelope exceeded 1400° C, but the envelope made of transparent yttria was not subjected to blackening and could be safely used for a long time at a temperature of 1400° C.

Table 2 shows the radiation efficiency of the high pressure sodium vapor discharge lamp using the above-mentioned transparent yttria envelope and that using the transparent alumina envelope. It is seen from this Table that the discharge lamp made of transparent yttria has a radiation efficiency of about 6 to 14 lm/W higher than that of the comparative lamp.

TABLE 2

| Envelope            | Lighting Conditions |                  | Efficiency            |                   |
|---------------------|---------------------|------------------|-----------------------|-------------------|
|                     | Lamp voltage (V)    | Lamp current (A) | Total light flux (lm) | Efficiency (lm/w) |
| Transparent yttria  | 91.0                | 5.05             | 44,610                | 116.3             |
| Transparent yttria  | 91.0                | 5.05             | 46,800                | 120.0             |
| Transparent yttria  | 91.0                | 5.07             | 47,750                | 124.0             |
| Transparent alumina | 100                 | 4.74             | 45,650                | about 110         |

FIG. 2 shows the relation between the grain size and inline transmission of the transparent yttria sintered body produced by the above process. It is seen from this Figure that, with the grain size more than 0.1 mm, the in-line transmission exceeds 40 percent, which means that the transparency of the sintered body is satisfactory for practical applications. However, with the grain size more than 5 mm, the sintered body is subject to cracks and a coarse grain boundary, although the data are not shown in FIG. 2. Therefore, the grain size less than approximately 5 mm is usually preferred.

It will be apparent from the above description that a high pressure sodium vapor discharge lamp using a transparent yttria envelope in accordance with the present invention has excellent sodium resistance and radiation efficiency as compared to the conventional sodium vapor discharge tube using a transparent alu-

TABLE 1

| Samples                                           | Treatment in Sodium-saturated Vapor |   | Appearance After Treatment Time (hours) | X-ray Analysis |
|---------------------------------------------------|-------------------------------------|---|-----------------------------------------|----------------|
|                                                   | Temp. (°C)                          |   |                                         |                |
| (This invention: pure yttria)                     | 1200                                | 3 | Unchanged                               | Yttria         |
| (Comparative: transparent alumina)                | 1200                                | 3 | Large cracks, opaque                    | γ-alumina      |
| (Comparative: yttria containing thorium Yttrolox) | 1200                                | 3 | Devitrification                         | —              |

mina or Yttralox envelope. Moreover, it has a lesser blackening and a longer service life than the above-mentioned conventional discharge tube and has a great practical utility.

It is usually preferred to have the thickness of both ends 11 of the envelope 1 shown in FIG. 1 larger than that of the outer region thereof as seen in FIG. 3. With the envelope of the uniform thickness, the outer surface of both ends of the envelope is preferably coated (see FIG. 4) with powdered heat-resistant material 12, such as alumina or yttria, so that the envelope may have a lower heat conductivity in the end portions than in the central zone. By this measure, stabilized discharge characteristics can be obtained as a result of obviating a temperature decrease at the end portions of 15 the envelope. As the powdered heat-resistant material to be coated on the outer surface of the end portions of the envelope, it is preferred to use oxides which have a thermal conductivity less than yttria and are chemically stable at operating temperatures. In addition, a 20 powdered heat-resistant material is preferably coated around outside of the opposite ends of the envelope up to the height of the electrodes.

What we claim is:

1. A high pressure sodium vapor discharge lamp 25 comprising:  
a tubular elongated envelope of sintered polycrystalline yttria consisting of corrosion resistant yttrium oxide and having an average grain size of 0.1 to 5 mm, said envelope having a pair of electrodes 30

sealed into opposite ends, and an ionizable medium including sodium vapor sealed within said envelope.

2. The high pressure sodium vapor discharge lamp 5 according to claim 1, in which said envelope has a heat resistant oxide layer coated on the outer sides of opposite ends thereof.

3. The high pressure sodium vapor discharge lamp 10 according to claim 2, in which said heat resistant oxide layer is selected from the group consisting of alumina and yttria.

4. The high pressure sodium vapor discharge lamp according to claim 1 wherein the thickness of the ends of said envelope in which said electrodes are sealed is greater than the thickness of the side of said envelope.

5. The high pressure sodium vapor discharge lamp according to claim 1 wherein a powdered heat-resistant material is coated on the outside of the opposite ends of said envelope up to the height of the electrodes sealed therein.

6. The high pressure sodium vapor discharge lamp according to claim 1, in which the corrosion resistant yttrium oxide of said envelope has an average grain size of 0.2 mm to 5 mm.

7. The high pressure sodium vapor discharge lamp according to claim 1, in which the corrosion resistant yttrium oxide of said envelope has an average grain size of 0.3 mm to 5 mm.

\* \* \* \* \*